# EUROPEAN PATENT SPECIFICATION

(11) **EP 2 871 283 B1**
(45) Date of publication and mention of the grant of the patent: **07.03.2018**
(21) Application number: 14460082.2
(22) Date of filing: 05.11.2014
(51) Int. Cl.: D21H 19/06, B41M 5/00, B41M 5/52, D21H 19/84, D21H 21/16

(54) **Ink-jet paper coating**
Tintenstrahlpapierbeschichtung
Revêtement de papier d'impression à jet d'encre

(30) Priority: 06.11.2013 PL 40594313
(43) Date of publication of application: 13.05.2015
(73) Proprietor: Arctic Paper Kostrzyn Spólka Akcyjna, 66-470 Kostrzyn nad Odra (PL)
(72) Inventor: Rawdanis, Janusz, 66-470 Kostrzyn nad Odra (PL); Marianczyk, Grzegorz, 91-088 Lódz (PL)
(74) Representative: Zielinski, Wojciech Leszek

(56) References cited:
- US-A1- 2009 297 738
- US-A1- 2012 019 587

## Description

The present invention relates to a paper coating for ink-jet printing.

Ink-jet printing, a technique pioneered during the second half of twentieth century, has created a need for paper of appropriate quality. During the last years of last century, special coatings designed for ink acceptance during printing were applied to improve print quality. The aim was achieved by hydrophilic coatings applied onto paper ground, using silica gel, polyvinyl alcohol and/or carboxymethylcellulose plus low molecular weight cationic polymer (e.g. modified polyethylenimine, polyvinylamine, condensation product of organic amides with formaldehyde, polyacrylamide) [Handbook of Paper and Board. Ed. H. Holik, WILEY-VCH Verlag GmbH & Co. KgaA, 2006, Weinheim, pp. 98-99]. Patent and specialist literature provide numerous versions of ink-jet paper coatings.

A paper ground for ink-jet printing with a cationic two-component surface coating is known from patent description US4,554,181. Cationic polymers applied in that invention characterises in that the cationic groups are available for anionic component of ink dye(s). The other source of cations are salts of a metal from group II, III or the Transition Metals of the Periodic Table of Elements of solubility greater than 5 g in 100 ml of water at 23°C. Due to tend to colour the paper, salts of Fe²⁺, Fe³⁺ and Cu²⁺ are scarcely useful. It was revealed that salts of strong acids (including hydrochloric acid) are capable of insolubilising anionic ink components, but the anionic parts of the strong acids accelerate paper degradation.

A coating for ink-jet paper is known for Japanese patent application description JP 2001315433, which consists of 2-10 parts by weight of inorganic electrolyte (preferably sodium chloride), 0-100 parts by weight of porous absorbing material (e.g. silica particles), and up to 100 parts by weight hydrophilic or vinyl acetal resin. The mixture is to be prepared onto a polyethylene foil and then transferred onto a paper.

A paper coating for ink-jet printing of hydrophilic properties according the invention, comprising of sodium aluminosilicate, sodium chloride, polyvinyl alcohol, aliphatic polyamine and polyaluminum chloride, characterises in that weight ratio of sodium chloride and polyaluminum chloride to aliphatic polyamine is 9.6 : 1. The coating is applied by a machine on a paper ground on one- or two-sides.

Unexpectedly, despite so high concentration of chlorides and sodium, a paper covered with the coating according to the invention is durable on one hand, and it provides good printing quality on the other hand. In addition, it is suitable for direct, mechanical applying on a paper with a standard machines. In laboratory tests on papers for ink-jet printing the following parameters were recorded: mottling, show-through, bleeding and optical density. Paper with the coating according to the invention was produced on a size press of a papermaking machine. Assessment of coatings consisted in evaluation of printouts using:
a) industrial inks INK JET (OCE) and a piezoelectric head of an office printer (Epson Stylus),
b) industrial printer Kodak Versmark,
c) industrial printer OCE.
The results are presented in a table and charts (F 83 - paper with the coating according to the invention, APP - standard paper, Mondi - a reference paper for ink-jet printing, CL3 - other tested product): The results confirm a printing quality comparable with those of the reference paper for ink-jet printing. No accelerated degradation was found.

The invention is illustrated by the following exemplary embodiment.

Example. Water is to be poured into a mixer with a high-speed stirrer at amounts depending on demanded concentration of the coating mixture, and than the ingredients are added gradually at the indicated amounts:

| Ingredient | Commercial name | Amount of a dry substance in g/100 g of the mixture | Weight percentage of all ingredients |
|---|---|---|---|
| Sodium aluminosilicate | Zeocros PF | 2 | 16.49% |
| Sodium chloride | evaporated salt | 6.25 | 51.54% |
| Polyvinyl alcohol | PVOH BP-05 | 3 | 24.74% |
| Aliphatic polyamine | CATIOFAST 160 | 0.67 | 5.50% |
| Polyaluminum chloride | PAX 18 | 0.21 | 1.73% |

Every ingredient shall be added as soon as a previous is completely dissolved in the mixture. A paper sheet is to be covered with the mixture with a papermaking machine or with a covering machine on one or two sides. Paper density of the produced paper is 70 - 160 g/m², and coating density is 2-4 g/m².

## Claims

1. A paper coating for ink-jet printing of hydrophilic properties, applied on one or two sides of a paper sheet, comprising of sodium aluminosilicate, sodium chloride, polyvinyl alcohol, aliphatic polyamine and polyaluminum chloride **characterised in that** weight ratio of sodium chloride and polyaluminum chloride to aliphatic polyamine is 9.6 : 1

## Patentansprüche

1. Eine Papierbeschichtung für den Tintenstrahldruck mit hydrophilen Eigenschaften, auf eine oder beide Seiten eines Papierblattes angewandt, bestehend aus Natriumaluminosilikat, Natriumchlorid, Polyvinylalkohol, aliphatischem Polyamin und Polyaluminiumchlorid, **gekennzeichnet dadurch, dass** das Gewichtsverhältnis von Natriumchlorid und Polyaluminiumchlorid zum aliphatischen Polyamin 9.6 : 1 beträgt.

## Revendications

1. Un revêtement de papier pour imprimantes à jet d'encre ayant des propriétés hydrophiles, appliqué sur une des deux faces d'une feuille de papier, composé d'aluminosilicate de sodium, d'alcool polyvinylique, de chlorure de sodium, de polyamine aliphatique et chlorure de polyaluminium qui se **caractérise par le fait que le rapport** en poids du chlorure de sodium et du chlorure de polyaluminium à la polyalumine aliphatique est de 9,6 : 1
